

## UNITED STATES PATENT OFFICE

2,605,775

PROCESS OF TREATING COLD ROLLED  
STRAIGHT CHROME TYPE STAINLESS  
STEELJoseph C. Kientz, Jr., Carnegie, Pa., assignor to  
Superior Steel Corporation, Pittsburgh, Pa., a  
corporation of VirginiaNo Drawing. Application February 21, 1947,  
Serial No. 730,196

6 Claims. (Cl. 134—3)

1

This invention relates to the treatment of cold rolled straight chrome type stainless steel and particularly to the annealing and pickling of such steel. It relates more particularly to a process of treating cold rolled straight chrome type stainless steel which makes feasible the batch annealing of such steel, as, for example, between cold reduction steps.

In the production of cold rolled straight chrome type stainless steel it is customary to cold roll hot rolled strip with intermediate continuous annealing and pickling steps. For example, if cold rolled straight chrome type stainless steel .018 inch in thickness is desired a customary way of producing such steel is to cold roll hot rolled strip .125 inch thick to about .060 inch in thickness, continuously anneal and pickle, then cold roll to about .032 inch in thickness, then again continuously anneal and pickle, then cold roll to final thickness and then for a third time continuously anneal and pickle. The continuous annealing and pickling steps are desirable because the oxide formed during annealing in that fashion is removable by pickling with the ordinary commercial pickling acids. However, a disadvantage is that the continuous annealing and pickling equipment is expensive and has to be used a plurality of times on the same strip. This means that for quantity production a considerable amount of continuous annealing and pickling equipment must be available.

I have discovered another way of producing cold rolled straight chrome type stainless steel not requiring the use of continuous annealing and pickling equipment. I have discovered that with a particular after treatment it is possible to substitute a batch anneal for the conventional continuous anneal.

It has heretofore been considered not feasible to batch anneal cold rolled straight chrome type stainless steel because when such steel is batch annealed there is formed thereon a film of oxide not satisfactorily removable by commercial pickling acids. The oxide is a tenacious chromic oxide which is insoluble in acids ordinarily used for commercial pickling such as sulphuric and nitric-hydrofluoric acids. While this chromic oxide film can be dissolved if the steel is treated by a special caustic reagent such, for example, as sodium hydride or molten sodium hydroxide containing an oxidizing agent prior to its treatment with acid, use of those reagents requires special equipment and is otherwise undesirable.

I have discovered that cold rolled straight chrome type stainless steel can be satisfactorily

produced on a commercial scale by substituting a batch anneal for the conventional continuous anneal if the steel is subjected to a treatment following the batch anneal and prior to the subsequent pickling treatment to fracture the tenacious oxide which is formed during the batch anneal. I find that if that oxide is fractured or cracked it is thereby rendered removable by the usual commercial pickling acids, e. g., by pickling successively in sulphuric and nitric-hydrofluoric acids. Apparently the pickling acids find their way through the fractures or cracks in the oxide film and by action at the contiguous surfaces of the steel and the oxide film partially dissolve the film and cause the undissolved portion to become separated from the steel. The undissolved film drops off in small pieces and settles at the bottom of the pickling tank from which it may be cleaned out.

20 The fracturing or cracking of the tenacious chromic oxide film formed by the batch annealing of cold rolled straight chrome type stainless steel may be effected by stretching the steel whereby to cause fracturing of the relatively unelastic film. I find it desirable to stretch the steel by cold rolling it. Only a single very light skin pass in a cold rolling mill is necessary to cause sufficient fracture or rupture of the oxide film to permit its effective removal by the ordinary commercial pickling acids. A reduction in gauge of the order of one or two thousands of an inch or less in very thin cold rolled straight chrome type stainless steel is ordinarily sufficient to effectively fracture the oxide film. It is preferable that the steel be subjected to the light skin pass when it is in dry condition.

The cold rolled straight chrome type stainless steels to which my invention is applicable are those containing chromium in about the range 10-30% and not containing a substantial percentage of nickel. Ordinarily such steels will contain carbon in about the range .01-1.2%. An example of a steel to which my invention is applicable is:

|            | Percent |
|------------|---------|
| Carbon     | .1      |
| Manganese  | .5      |
| Silicon    | .3      |
| Phosphorus | .02     |
| 45 Sulphur | .02     |
| Chromium   | 17      |
| Nickel     | .3      |

As an illustration of a procedure according to my invention for the production of cold rolled

straight chrome type stainless steel, I may hot roll a billet of straight chrome type stainless steel to about .125 inch in thickness, batch anneal and pickle in the usual way for hot rolled strip, cold roll to about .060 inch in thickness, batch anneal, skin pass in a cold rolling mill (reducing the gauge say .002 inch), pickle successively in sulphuric acid and nitric-hydrofluoric acid, cold roll to about .032 inch in thickness, batch anneal, skin pass in a cold rolling mill (reducing the gauge say .002 inch), pickle successively in sulphuric acid and nitric-hydrofluoric acid, cold roll to about .018 inch in thickness, batch anneal, skin pass in a cold rolling mill (reducing the gauge say .001 inch) and pickle successively in sulphuric acid and nitric-hydrofluoric acid. The steel may be pickled either in the coil or continuously or after shearing into relatively short lengths. If it is pickled in the coil the convolutions of the coil should be slightly separated to permit adequate ingress of the pickling acids. I prefer to pickle the steel continuously. This may be done either as a combined continuous operation with the cold rolling step and immediately following the cold rolling or as a separate step, the steel being coiled following cold rolling and then uncoiled prior to pickling. In pickling the steel is preferably treated successively with sulphuric acid and nitric-hydrofluoric acid.

As above explained the oxide film cracking step enables the ordinary commercial pickling acids to effectively remove the tenacious chromic oxide film formed on the cold rolled straight chrome type stainless steel in batch annealing, rendering unnecessary the use of caustic reagents and the equipment needed for treatment therewith.

While I have described a present preferred method of practicing the invention it is to be distinctly understood that the invention is not limited thereto but may be otherwise variously practiced within the scope of the following claims.

I claim:

1. In the treatment of cold rolled straight chrome type stainless steel containing chromium in about the range 10-30% which has formed thereon a film of oxide such as is formed by batch annealing and which is not satisfactorily removable by pickling successively in sulphuric and nitric-hydrofluoric acids, the steps of stretching the steel by cold rolling it, thereby forming cracks in said film, and pickling the steel successively in sulphuric and nitric-hydrofluoric acids which after the first mentioned step is effective for satisfactorily removing the film.

2. In the treatment of cold rolled straight chrome type stainless steel containing chromium in about the range 10-30% which has formed thereon a film of oxide such as is formed by batch annealing and which is not satisfactorily removable by pickling successively in sulphuric and nitric-hydrofluoric acids, the steps of forming cracks in said film by stretching the steel and pickling the steel successively in sulphuric and nitric-hydrofluoric acids which after the first mentioned step is effective for satisfactorily removing the film.

3. In the treatment of cold rolled straight chrome type stainless steel containing chromium

in about the range 10-30% which has formed thereon a film of oxide such as is formed by batch annealing and which is not satisfactorily removable by pickling successively in sulphuric and nitric-hydrofluoric acids, the steps of subjecting the steel to a light skin reducing pass in a cold rolling mill, thereby forming cracks in said film, and pickling the steel successively in sulphuric and nitric-hydrofluoric acids which after the first mentioned step is effective for satisfactorily removing the film.

4. In the treatment of cold rolled straight chrome type stainless steel containing chromium in about the range 10-30% which has formed thereon a film of oxide such as is formed by batch annealing and which is not satisfactorily removable by pickling successively in sulphuric and nitric-hydrofluoric acids, the steps of stretching the steel by cold rolling it, thereby forming cracks in said film, and continuously with said cold rolling pickling the steel successively in sulphuric and nitric-hydrofluoric acids which after the first mentioned step is effective for satisfactorily removing the film.

5. In the treatment of cold rolled straight chrome type stainless steel containing chromium in about the range 10-30% which has formed thereon a film of oxide such as is formed by batch annealing and which is not satisfactorily removable by pickling successively in sulphuric and nitric-hydrofluoric acids, the steps of stretching the steel by cold rolling it, thereby forming cracks in said film, coiling the steel after said cold rolling and thereafter uncoiling and continuously pickling the steel successively in sulphuric and nitric-hydrofluoric acids which after the first mentioned step is effective for satisfactorily removing the film.

6. In the treatment of cold rolled straight chrome type stainless steel containing chromium in about the range 10-30% which has formed thereon a film of oxide such as is formed by batch annealing and which is not satisfactorily removable by pickling successively in sulphuric and nitric-hydrofluoric acids, the steps of forming cracks in said film by stretching the steel and pickling successively in sulphuric and nitric-hydrofluoric acids the steel in coil form with the convolutions of the coil slightly separated to permit free access of the pickling acid, which pickling after the first mentioned step is effective for satisfactorily removing the film.

JOSEPH C. KIENTZ, JR.

REFERENCES CITED

The following references are of record in the file of this patent:

UNITED STATES PATENTS

| 60. Number    | Name        | Date          |
|---------------|-------------|---------------|
| 394,613       | Dempster    | July 23, 1908 |
| 1,392,780     | Marsh       | Oct. 4, 1921  |
| 1,567,143     | Hay         | Dec. 29, 1925 |
| 1,765,498     | Naugle      | June 24, 1930 |
| 65. 1,837,159 | Fellows     | Dec. 15, 1931 |
| 2,340,461     | Gage et al. | Feb. 1, 1944  |
| 2,347,742     | Keene       | May 2, 1944   |